

July 17, 1956

J. B. STUCKER ET AL

2,755,248

## ALKALINE EARTH METAL BASE GREASES AND THEIR PREPARATION

Filed Oct. 16, 1951



**INVENTORS**

BY JOSEPH B. STUCKER  
ERNEST T. FRONCZAK

Edward H. Lang  
ATTORNEY

1

2,755,248

**ALKALINE EARTH METAL BASE GREASES AND THEIR PREPARATION**

Joseph B. Stucker, Des Plaines, and Ernest T. Fronczak, Crystal Lake, Ill., assignors to The Pure Oil Company, Chicago, Ill., a corporation of Ohio

Application October 16, 1951, Serial No. 251,482

4 Claims. (Cl. 252—40)

This invention relates to grease compositions and to a method for their preparation. More particularly, this invention relates to a semi-solid grease composition containing a metal soap gelling agent, solvent refined lubricating oil, and a solvent extract from the manufacture of lubricating oil stocks.

Greases, being physically gel systems of fluid lubricant and gelling agents, are normally prepared by pressure saponification of fat stock, followed by dehydration of the metal soap, cut-back with mineral oil, hydration, and reduction to the consistency grade desired. The principal characteristics of greases which bear importance as far as manufacture and use are concerned, comprise consistency, consistency stability, melting or flow point, yield value, the free acid or alkali content, and stability in storage and use. Numerous techniques have been developed for both batch and continuous methods of grease preparation. However, these techniques provide for little flexibility in the grease composition for a given type of grease and are built around expensive low viscosity index lubricating oil fractions. Also, prior methods are applicable to those types of grease wherein the attainment of a stable gel structure presents little difficulty as, for example, aluminum or lithium soap greases. It is generally considered that it is more difficult to attain good texture, high yield values, and stability in the manufacture of soda soap, soda-lime soap, and lime-base greases than other types of grease. Those processes directed to the preparation of lime-base greases require tedious processing techniques, employing expensive lubricating oil stocks, and often depend upon expensive additives, as high molecular weight synthetic polymers, to attain the desired results. Automotive chassis greases have been prepared using Gulf Coast type lubricating oils which are entirely satisfactory performance-wise, but the cost of manufacture is high and the processing technique often tedious. In addition no flexibility of the composition is attained whereby chassis greases can be prepared for use in divergent climatic conditions requiring stringent viscosity/temperature relationships in the grease using prior methods of manufacture.

Another difficulty with existing grease manufacture processes and compositions is that they are not amenable to the use of solvent refined lubricating oils unless low viscosity neutral fractions are used, and even then the required soft, fine grain texture and compatibility with metal soaps is lacking. Solvent refined oils have not generally been used in the manufacture of greases, especially lime-base greases because of the incompatibility of the oil with the lime soaps and the fact that the viscosity of the solvent refined oils cannot be varied within the broad limits necessary to form greases operable under extremes of climatic conditions. If it is attempted to raise the viscosity index of the solvent refined oils by employing blends of solvent refined neutral stocks and high viscosity index solvent refined bright stocks, the result is a destruction of the gel structure of the grease.

2

The primary object of this invention is to provide a method of manufacturing greases and compositions therefore which overcome these difficulties. It has been found that grease compositions may be prepared using solvent refined lubricating oil stocks by including in the formulation substantial portions of solvent extract from the solvent refining of lubricating oils. Greases formulated in accordance with this invention using the techniques herein described and the compositions disclosed not only eliminate the foregoing difficulties but also meet the most exacting specifications. Greases formulated in accordance with this invention do not need expensive additives or expensive highly refined lubricating oil bases as a part of the composition in order to meet the required viscosity/temperature relationships for various climatic conditions, the tackiness and water-insolubility required of a chassis lubricant, or the flexibility required for economic production. The diagram is a simplified representation of the apparatus employed and the flow of ingredients in conducting the present process.

One of the objects of this invention is to provide grease compositions containing alkaline earth metal and alkali metal soaps, or alkaline earth metal soaps wherein the mineral lubricating oil base is flexible as concerns its physical characteristics.

An object of this invention is to provide a grease composition in which the mineral lubricating oil base comprises the less expensive solvent refined lubricating oils in combination with the solvent extract from lubricating oil fractions.

Another object of this invention is to provide a lime-base grease composition in which the viscosity of the mineral lubricating oil base can be varied from about 150 SUS at 100° F. to about 5000 SUS at 100° F.

Another object of this invention is to provide a lime-base chassis grease composition which exhibits desired properties of pumpability, tackiness, adhesiveness, and consistency stability.

Another object of this invention is to provide a lime-base grease composition which includes a high viscosity index mineral lubricating oil base and, therefore, displays improved viscosity/temperature characteristics.

Another object of this invention is to provide a method for compounding grease compositions using solvent refined mineral lubricating oil stocks.

The present invention contemplates a grease which has a small moisture content for use at temperatures up to 150° F., under medium pressures and medium speeds and which contains a substantial amount of a solvent extract from a mineral lubricating oil and a small amount of lime-soda soaps. The solvent extracts used in accordance with this invention are obtained during the manufacture of neutral and bright lubricating oil stocks.

In a typical operation, desalted crude oil is first charged to a distillation unit where straight run gasoline, two grades of naphtha, kerosene, and virgin distillate are taken off, leaving a reduced crude residue. The reduced crude is continuously charged to a vacuum distillation unit where three lubricating oil distillates are taken off as side streams, a light distillate is taken off as overhead, and a residuum is withdrawn from the bottom of the tower. This residuum is charged to a propane deasphalting unit wherein propane dissolves the desirable lubricating oil constituents and leaves the asphaltic materials. A typical vacuum residuum charge to the propane deasphalting unit may have an API gravity of 12.9°, viscosity SUS at 210° F. of 1249, flash 585° F., fire 650° F., C. R. of 13.9 weight per cent and is black in color. The deasphalting oil may have an API gravity of 21.5° to 21.8°, viscosity SUS at 210° F. of 165-175, NPA color 6-7, flash 575° F., fire 640° F., and C. R. of 1.7-2.0.

The deasphalted oil and various lubricating oil distillates from the reduced crude are separately subjected to solvent extraction for the separation of non-aromatic from aromatic constituents. The refined oil or "raffinate" from such processes is used as blending stocks and the solvent extract, containing the undesirable aromatic constituents, is the material found useful in accordance with this invention.

For example, a Van Zandt crude oil with an API gravity of 33.1 was topped to remove such light fractions as gasoline, naphtha, kerosene, and a light lubricating distillate. The vacuum residue was a reduced crude having a viscosity of 1251 SUS at 210° F., 2.2 per cent sulfur, and an API gravity of 12.6. After propane deasphalting, the oil had a viscosity of 174 SUS at 210° F. and an API gravity of 21.7. This deasphalted oil was treated with phenol to produce a raffinate from which an aviation lubricating oil may be produced. The extract phase from this phenol treatment is ready for use in preparing greases in accordance with this invention.

Other solvents than phenol may be used to obtain the extraction product used in accordance with this invention; for example, furfural or the Duo-Sol solution comprising liquid propane, phenol, and cresol may be used. When using phenol, it is possible to vary the characteristics of the extraction product considerably by adjustment of the amount of water present. A low V. I. cut may be obtained by using a water solution of phenol during the extraction and a high V. I. cut may be obtained by using anhydrous phenol. Following are the physical characteristics of typical extraction products from bright stock from Van Zandt crude oil which may be used in accordance with this invention.

TABLE I  
Physical characteristics of phenol extracts

| Extract No. | API Gravity | Viscosity/100° F. | Viscosity/130° F. | Viscosity/210° F. | V. I. | Pour, ° F. | Percent C. R. | Percent Sulfur |
|-------------|-------------|-------------------|-------------------|-------------------|-------|------------|---------------|----------------|
| 1-----      | 11.1        | 23,319            | 4,750             | 282               | -40   | +55        | 7.2           | 2.66           |
| 2-----      | 15.4        | 15,000            | 285               | +39               | -1    | +80        | 4.7           | 2.27           |
| 3-----      | 12.6        | 36,410            | 4,310             | 310.1             | +27   | +90        | 4.7           | 2.2            |
| 4-----      | 14.6        | 19,500            | 4,305             | 313               | +5    | +60        | 4.13          | 2.33           |
| 5-----      | 15.4        | 32,500            | 372               | +27               | +80   | -          | 2.18          |                |
| 6-----      | 13.7        | 25,000            | 5,400             | 355               | +27   | -          |               |                |
| 7-----      | 8.6         | 145,000           | 19,000            | 616               | <0    | +70        |               |                |

The extracts shown in Table I are merely illustrative and the invention is not to be limited thereby. It is to be understood that any solvent extract from the refining of lubricating oils for the purpose of separating non-aromatic and aromatic hydrocarbons will apply and be useful in the present invention, provided it can be blended with a lubricating oil to form the proper viscosity blend for grease manufacture.

By using solvent extracts in substantial quantity in grease compositions, the processing technique is simplified and the resulting products display the desired viscosity/temperature relationships, pass the commercial requirements of consistency stability, display the required characteristics of pumpability, tackiness, and require less metal soap in the composition to give a good grease consistency. Furthermore, greases prepared in accordance with this invention are adhesive to metal parts, water-insoluble, and provide excellent lubrication at temperatures up to 150° F. or as low as -30° F.

The following formula sets forth the general limits of the ingredients of the new grease. This formula is not to be considered as restrictive, since the proportions may be varied so long as the characteristics and properties of the compositions are not departed from in any substantial manner. Grease compositions prepared in accordance with this invention may be of any consistency from 0 (worked penetration 355-385) to 5 (worked penetration 130-160).

|                   | Percent by weight |
|-------------------|-------------------|
| Fatty acids       | 8-9               |
| Hydrated lime     | 1.5-1.7           |
| Caustic           | .01-0.20          |
| 5 Solvent extract | 60-65             |
| Mineral oil       | 24-30             |
| Water             | 0.2-35            |

A specific example of a grease composition compounded in accordance with this invention comprises:

|                                          | Percent by weight |
|------------------------------------------|-------------------|
| Animal fatty acids                       | 8.40              |
| Hydrated lime                            | 1.60              |
| Sodium hydroxide                         | 0.06              |
| 15 Phenol extract from bright stock mfr. | 62.77             |
| Neutral lubricating oil                  | 26.89             |
| Water                                    | 0.28              |

The grease of the above formula shows the following characteristics and tests:

|                                                                                   |         |      |
|-----------------------------------------------------------------------------------|---------|------|
|                                                                                   |         |      |
| 20 Soda soap                                                                      | percent | 0.8  |
| Lime soap                                                                         | do      | 9.0  |
| Mineral oil                                                                       | do      | 89.0 |
| Free acid                                                                         | do      | .00  |
| 25 Free alkali                                                                    | do      | .03  |
| Unworked consistency (A. S. T. M.)                                                |         | 294  |
| Worked consistency (A. S. T. M.)                                                  |         | 290  |
| Apparent viscosity in poises at 77° F. with rates of shear (sec. <sup>-1</sup> ): |         |      |
| 30 10                                                                             |         | 720  |
| 100                                                                               |         | 162  |
| 1,000                                                                             |         | 53   |
| 10,000                                                                            |         | 28   |
| Consistency stability                                                             |         | Good |

The mineral oil used was a blend of Mid-Continent solvent refined neutral and heavy stock having a viscosity of about 2400 SUS at 100° F., V. I. 45, and an API gravity of 20.5. If the viscosity of the mineral oil is increased to as much as 3000 or 4000 SUS at 100° F., the apparent viscosity of the finished grease at high shear rates (10,000 sec.<sup>-1</sup>) can be increased appreciably above 55 the 28 poises shown above. The fatty acids referred to include both animal and vegetable fatty acids, as stearic acid, palmitic acid, etc. The above grease qualifies as No. 2 consistency summer chassis grease, is readily pumped through standard grease pumping equipment and forced through the various fittings of an automobile chassis. It will adhere to the bearing surfaces at temperatures up to 150° F. and is not affected by water. In testing this grease, it was found that the apparent viscosity at high shear rates is dependent on the mineral oil 60 viscosity and soap content of the grease while the apparent viscosity at low shear rates is dependent on the yield, that is, the per cent by weight of soap needed to form a grease of a certain consistency.

In general, the process of formulating greases in accordance with the present invention comprises heating and agitating the solvent extract in a mixing chamber; preparing a slurry of a portion of the lubricating oil and lime; preparing a solution of caustic soda, adding the caustic soda solution to the phenol extract at a temperature 75 of about 160° F. while continuing the agitating and

heating thereof; bringing the solvent extract to about 180° F. and then slowly adding a portion of the lime slurry; continuing the heating and allowing the mixture to reach a maximum temperature of 203° F.; holding the mixture at this temperature for a period of time while adding the balance of lubricating oil, which is followed by the addition of the fatty acids; and finally the remaining portion of the lime slurry is added.

After checking the free alkalinity and making corrections to bring the free alkali in the range of 0.01 to 0.10 per cent, the agitation is continued for about 15 minutes. The samples are drawn and quick chilled to determine the worked penetration. Then the mixture is cut back with lubricating oil stock and the balance of phenol extract until a particular "quick-chilled" penetration is achieved. The grease is then ready for drawing and packaging.

Referring to the diagram, lubricating oil stock is introduced to lime-slurry mixer 1 by means of line 2. Mixer 1 is fitted with stirrer 3 and valve 4 controlling the flow of slurry to pump 5. Pump 5 is connected to dispersion and recirculating system 6, comprising eductor 7, by-pass 8, disperser 9, and recycle line 10. Line 11 serves as a take-off for completed slurry conveying it to reaction kettle 12, fitted with stirrer 13 and caustic inlet 14.

Following the diagram, a detailed description of the process of the present invention is presented based on a 10,000 pound batch of grease (10,168 pounds total). The components for this example composition are:

TABLE II

| Component                                  | Pounds |
|--------------------------------------------|--------|
| Animal fatty acids                         | 855    |
| Hydrated lime                              | 163    |
| Caustic soda                               | 7      |
| Phenol extract                             | 6,380  |
| Viscosity 200 SUS at 100° F., MCSR Neutral | 2,735  |
| Water                                      | 28     |

The kettle 12 was first charged with 6,380 pounds of phenol extract (about 750 gallons at 60° F.) and agitation through stirrer 13 and heat are applied. About 500 pounds of 200 vis neutral oil were added to the slurry mixer tank. About 163 pounds of lime were added through the eductor 7. Agitation of the slurry mixer tank was begun by means of stirrer 3 and valve 4 opened to start the dispersion and recirculating system 6. The valves and by-pass 8 were then adjusted to gradually pull the lime into the system, through the disperser 9 and through recycle line 10 into tank 1. Seven pounds of caustic soda were dissolved in 28 pounds of water and the solution added through line 14 to kettle 12 when the phenol extract therein had reached a temperature of about 160° F. Agitation and heating were continued. When the extract reached 180° F., about 80 pounds of lime/oil slurry from dispersion system 6 were added through line 11. Heating and agitation in kettle 12 were continued, allowing the mixture to reach a maximum temperature of about 203° F.

The mixture was maintained at a temperature of 200° F. to 203° F. for about 15 minutes, during which time about 1,735 pounds of 200 vis neutral lubricating oil were added. 855 pounds of animal fatty acids were then added to the mixture in kettle 12, and the temperature adjusted to 200° F. to 203° F. The remainder of the lime/oil slurry in tank 1 was next added to the contents of kettle 12. Immediately following this step, it is well to wash the slurry mixer tank with 500 pounds of 200 vis neutral, preferably in two stages so that hang-up of lime within the system is minimized.

The mixture in kettle 12 was agitated at 200° F. to 203° F. for about 30 minutes after the last wash oil had been added from the previous step. At this stage in the process, it is convenient to check the free alkalinity which should be maintained within the range of 0.01 to

0.10 per cent. If acid or lime are necessary to correct the alkalinity, the agitation is continued for 15 minutes to insure complete reaction. If no correction is necessary, the agitation is continued for one hour after the addition of the wash oil.

The progress of the grease formation should be determined by withdrawing a sample, quick-chilling, and determining the 60-stroke worked penetration. The sample should have a worked penetration of about 290 at this point. The entire batch was next cut back with 200 vis neutral lube oil and phenol extract to a quick-chill penetration of about 320 to 340. The grease is ready for packaging. The total time elapsed in the batch process is about three to three and one-half hours.

In order to further demonstrate the invention, a series of experimental grease batches were prepared using different mineral lubricating oil bases and different types of fat stock. Some batches were prepared using the ordinary cut-back method of pressure saponification of the fat stock followed by dehydration of the lime soap, cut back with mineral oil, hydration of the grease and reduction to consistency in the normal fashion. Other batches were prepared using a modified method wherein a portion of the mineral oil base and all the fatty acids are mixed and heated to 180° to 185° F., then the sodium hydroxide added as a 25 per cent aqueous solution. The balance of the mineral oil base was used to prepare a lime slurry (approximately one part by weight of lime and three parts of neutral oil). This lime slurry was added to the batch and the temperature raised to 200° F. The temperature was maintained at about 205° to 210° F. for about two hours and the remainder of water added. Solvent extract was then added over a period of about two hours and the temperature allowed to drop to 190° to 200° F., at which temperature the grease was drawn.

Still another method was employed, designated "special" in the table, wherein the procedure was to charge a portion of the neutral oil, all the fatty acids, and all the phenol extract to the grease kettle and the mixture was heated to about 160° F. or enough to melt the fatty acids. The caustic soda (as a 25 per cent solution) was added and the temperature slowly raised to about 230° F., agitation was continued and the temperature allowed to drop to about 205° F. Next, the lime slurry of neutral oil and lime heated to 200° to 205° F. was added and additional hot neutral oil used to flush out any remaining lime slurry from the lime slurry mixer. The kettle was maintained at about 200° to 210° F. for a period of one and one-half to two hours without exceeding 210° F. after the lime slurry was added. The batches were drawn at 190° to 200° F. This method is exemplified by batch number 13. Lastly, Table III shows batch 15 was prepared using the preferred method which has heretofore been described. These modifications in procedure were a matter of altering the ordinary cut-back method to obtain a process whereby a good grease having the desired characteristics could be prepared, using high viscosity solvent extracts with solvent refined oils, most economically and efficiently without the chance of failure to form a good grease.

From Table III it is apparent from batch numbers 1 and 5 that Gulf Coast oils may be readily used to compound lime-base greases using fatty acids or yellow grease (containing glycerides). Neutral stocks, bright stocks, or phenol extract alone, or phenol extract from the preparation of neutral stocks are difficult to handle in grease making and do not yield a product having the proper characteristics, as good grease structure without the presence of grain. This is shown by batches 2, 3, 4, 5, and 6. From phenol extract from the manufacture of bright stock (batch 7) formed a grainy grease and was difficult to hydrate. The addition of bright stock to a neutral stock (batch 8) completely disintegrated the gel structure. However, the combination of phenol extracts and neutral lubricating oil stocks of various viscosities

TABLE III

| No. | Weight Percent and Type of Mineral Oil                                         | Manufacturing Procedure | Type of Fat   | Percent Soap To Obtain Grease | Consistency |        | Free Acid or Alkali | Remarks                                                                                                                                                                                           |
|-----|--------------------------------------------------------------------------------|-------------------------|---------------|-------------------------------|-------------|--------|---------------------|---------------------------------------------------------------------------------------------------------------------------------------------------------------------------------------------------|
|     |                                                                                |                         |               |                               | Un-worked   | Worked |                     |                                                                                                                                                                                                   |
| 1   | 100% 2,046 Viscosity/100° F. Gulf Coast Oil.                                   | Cut-back                | Fatty acids   | 9.1                           | 328         | 328    | 0.03% Acid          | Good yield, good consistency and grease structure, meets desired apparent viscosity of 35-40 poises at 77° F. with 10,000 Sec <sup>-1</sup> shear rate, slight aeration.                          |
| 2   | 100% Viscosity 200 SUS at 100° F. Neutral.                                     | Modified                | do            | 15.0                          |             |        | 0.06% Alkali        | Poor yield, lumpy, hang-up on stirring paddles, grainy structure.                                                                                                                                 |
| 3   | 100% Intermediate V.I. Bright Stock.                                           | do                      | do            | 26.0                          |             |        |                     | Very soft grease, gel structure almost gone, low yield.                                                                                                                                           |
| 4   | 100% Viscosity 200 SUS at 100° F. Neutral.                                     | Cut-back                | Yellow grease | 26.0                          |             |        | 0.08% Alkali        | Difficult to hydrate, soft grainy grease, low yield.                                                                                                                                              |
| 5   | 100% 2,000 Viscosity/100° F. Gulf Coast Oil.                                   | do                      | do            | 10.5                          |             | 323    |                     | Good yield, good grease structure, meets desired apparent viscosity characteristics.                                                                                                              |
| 6   | 100% Phenol Extract from Neutral Stock Manufacture.                            | do                      | do            | 15.0                          |             |        |                     | Poor yield, very soft grease.                                                                                                                                                                     |
| 7   | 100% Phenol Extract #3                                                         | do                      | do            | 25.0                          |             |        |                     | Difficult to hydrate, grainy structure, low yield.                                                                                                                                                |
| 8   | 33% Viscosity 200 SUS at 100° F. Neutral, 67% 150 Viscosity 97 V. I. Brt. Stk. | do                      | Fatty acids   | 15.6                          | 386         | 375    | 0.17% Alkali        | Grease structure entirely disintegrated.                                                                                                                                                          |
| 9   | 65% Phenol Extract #1, 35% 200 Vis. Neut.                                      | do                      | Yellow grease | 15.0                          | 226         | 242    | 0.15% Acid          | Good grease structure, easy to hydrate, no grains.                                                                                                                                                |
| 10  | 65% Phenol Extract #3, 35% Viscosity 200 SUS at 100° F. Neut.                  | Modified                | Fatty acids   | 15.0                          |             |        | 0.20% Acid          | Fair grease structure, slight aeration.                                                                                                                                                           |
| 11  | 65% Phenol Extract #3, 35% Viscosity 200 SUS at 100° F. Neut.                  | do                      | do            | 13.0                          | 302         | 295    | 0.03% Acid          | Good grease structure, good yield.                                                                                                                                                                |
| 12  | 65% Phenol Extract #3, 35% Viscosity 200 SUS at 100° F. Neut.                  | do                      | do            | 11.0                          | 339         | 316    | 0.07% Acid          | Very good grease structure, excellent yield.                                                                                                                                                      |
| 13  | 65% Phenol Extract #4, 35% Viscosity 160/180 SUS at 100° F. Neut.              | Special                 | do            | 9.5                           | 306         | 311    | 0.09% Acid          | Good grease structure, good yield, no grains, consistency after 5,000 strokes 339 (84° F.).                                                                                                       |
| 14  | 65% Phenol Extract #3, 35% Viscosity 160/180 SUS at 100° F. Neut.              | Modified                | do            | 11.0                          | 308         | 311    | 0.05% Alkali        | Good grease structure, consistency after working 500 strokes 314; 1,000 strokes 326; 5,000 strokes 326 (Temp. 90° F.), apparent viscosity at 77° F. and a 10,000 Sec <sup>-1</sup> = 30.0 poises. |
| 15  | 70% Phenol Extract #3, 30% Viscosity 200 SUS at 100° F. Neut.                  | Preferred               | do            | 9.8                           | 294         | 290    | 0.03% Alkali        | Good grease structure and consistency stability, no foaming, no grains.                                                                                                                           |

proved to be the most satisfactory for both yellow grease and fatty acids, as evidenced by batches 9 to 14.

In preparing these grease compositions, it was observed that there was a tendency for the finished grease to be slightly acid. This is not deleterious and the degree of acidity or alkalinity can be adjusted during the final stages of preparation by extracting a sample, determining the per cent of acid or alkali and adding a small amount of alkali or acid to make the proper adjustment. It is generally preferred that the greases be slightly on the alkaline side, although this is not mandatory. The tendency of the grease compositions to be slightly acid may be accounted for by the presence of naphthenic acids in the solvent extracts used.

The yellow grease used in the above compositions has a saponification number of 192, an iodine value of 58, and showed on analysis considerable glyceride content along with about 12 per cent by weight of free fatty acids, calculated as oleic acid. The hydrated lime assayed at about 91 per cent calcium hydroxide. The fatty acids have a saponification number of from 200 to 208, iodine value of 50 to 57, and the fatty acid content ranges from 95.5 per cent to 100 per cent, calculated as oleic acid. The titer value °C. ranges from 40° to 41°.

Grease compositions have thus been described containing lime soaps and small amounts of soda-soaps. Calcium soaps may be incorporated as the alkaline earth metal soap with or without small amounts of alkali metal soaps, such as sodium, potassium, or cesium soaps. Lime base greases containing only lime-soaps may be prepared by the methods of this invention. As above stated, the fatty acids may be of animal, vegetable, or synthetic origin, and generally mixtures of saturated and unsaturated organic fatty acids having 10 or more carbon atoms to the molecule are contemplated. Those fatty acids are contemplated for use in this invention which form soaps yielding a gel structure which is stable and

free from graininess. The proportions of each of the ingredients may be varied within the limits disclosed without departing from the spirit of the invention. Likewise, the amount of dilution or cut-back in the final stages of preparation to attain the desired consistency may be varied within limits known to the art.

45 It has thus far been demonstrated that by employing the techniques of the present invention, there will be produced stable greases having consistencies, apparent viscosities, and consistency stabilities which are generally desired for greases useful as winter chassis lubricants, 50 summer chassis lubricants, cup greases, or hot mill or roll neck greases. Using the techniques herein disclosed, a soft grain grease is attainable, containing no lumps and the procedure is devoid of such processing difficulties as foaming and local overheating.

55 It is generally desirable that chassis greases, especially those to be used under different climatic conditions, exhibit certain prescribed pressure/viscosity characteristics for a designated consistency range. For example, a Number 1 consistency grease, which is known as a summer chassis grease, should have a worked penetration of 310 to 340, and should display the following pressure/viscosity characteristics:

|    | Viscosity (poises) at 77° F. | Shear Rate Sec. <sup>-1</sup> |
|----|------------------------------|-------------------------------|
| 65 | 100-200                      | 100                           |
|    | 50-80                        | 1,000                         |
|    | 25-35                        | 10,000                        |

70 Grease compositions prepared in accordance with this invention will display the above characteristics. It is realized that as the consistency grade increases, the apparent viscosity values at lower shear rates increase considerably. However, the apparent viscosity values at high shear rates will show only small increases. The

desired pressure/viscosity characteristics for winter chassis greases, cup greases, journal box greases, hot mill and roll neck greases can be also attained. Greases prepared using the described techniques do not become soft on being worked, nor do their gel structures disintegrate during use. The greases are easily pumped through chassis fittings and greasing equipment under divergent climatic conditions.

It has also been found that, by incorporating a certain combination of extreme pressure additives into greases prepared in accordance with this invention, a product is obtained having the extreme pressure characteristics necessary for heavy duty industrial uses. A grease meeting the Timken Roller Bearing Company's specifications for use on heavy duty steel mill roller bearing equipment may be prepared using lead naphthenate in combination with an additive marketed under the trade name of Stan-Add 48, which is a sulfurized terpene product deactivated at temperatures of about 200° to 250° F. to render it noncorrosive at 200° F. The sulfurized terpene is described in and may be made in accordance with United States Patent 2,445,983. Such grease meets the Timken Roller Bearing Company specifications for heavy duty use, including freedom from foreign constituents, fillers, etc., the required consistencies, noncorrosiveness to copper or steel at normal bearing temperatures, and the required extreme pressure qualities. This latter characteristic is demonstrated by the prevention of scoring on the Timken lubricant tester, using a minimum load of 33 pounds on the lever arm at a minimum rubbing speed of 400 feet per minute.

A series of experiments were conducted to demonstrate that grease compositions made in accordance with this invention may be further blended with a certain combination of extreme pressure additives to pass the Timken test. The results of these experiments are shown in the following Table IV.

TABLE IV

| Grease No. | Composition                                                                                                                          | Beam Load, Pounds                            | Test Rating                        |
|------------|--------------------------------------------------------------------------------------------------------------------------------------|----------------------------------------------|------------------------------------|
| 15.        | (Animal Fatty Acids.....<br>Hydrated Lime.....<br>Sodium Hydroxide.....<br>Phenol Extract.....<br>Lubricating Oil.....<br>Water..... | 8.4<br>1.6<br>0.06<br>62.75<br>26.89<br>0.28 | 25<br>33<br>-----<br>Do.           |
| 16.        | Grease #15.....<br>Dibenzyl Disulfide.....                                                                                           | 98.0<br>2.0                                  | 25<br>33<br>Do.                    |
| 17.        | Grease #15.....<br>Dibenzyl Disulfide.....                                                                                           | 94.0<br>6.0                                  | 33<br>Do.                          |
| 18.        | Grease #15.....<br>Tricresyl Phosphate.....                                                                                          | 98.5<br>1.5                                  | 25<br>Do.                          |
| 19.        | Grease #15.....<br>Tricresyl Phosphate.....                                                                                          | 95.0<br>5.0                                  | 25<br>Do.                          |
| 20.        | Chassis Grease A.....                                                                                                                | 100.0                                        | 25<br>Do.                          |
| 21.        | Chassis Grease A.....<br>(Tricresyl Phosphate.....                                                                                   | 98.5<br>1.5                                  | 25<br>Do.                          |
| 22.        | Chassis Grease A.....<br>Dibenzyl Disulfide.....                                                                                     | 96.0<br>4.0                                  | 25<br>Do.                          |
| 23.        | Chassis Grease A.....<br>Additive B.....                                                                                             | 99.0<br>1.0                                  | 33<br>Do.                          |
| 24.        | Chassis Grease A.....<br>Lead Naphthenate.....                                                                                       | 97.0<br>3.0                                  | 25<br>33<br>Do.                    |
| 25.        | Grease #15.....<br>Lead Naphthenate.....<br>Sulfur.....<br>Air-blown Asphalt.....                                                    | 79.0<br>10.0<br>1.0<br>10.0                  | 33<br>33<br>Pass.<br>Seizure.      |
| 26.        | Grease #15.....<br>Stan-Add 48.....<br>Lead Naphthenate.....                                                                         | 94.0<br>1.0<br>5.0                           | 33<br>33<br>Pass.<br>Do.           |
| 27.        | Grease #15.....<br>Lead Naphthenate.....<br>Stan-Add 48.....                                                                         | 94.5<br>5.0<br>0.5                           | 33<br>33<br>Do.<br>Do.             |
| 28.        | Grease #15.....<br>Lead Naphthenate.....<br>(Additive C.....                                                                         | 92.82<br>5.0<br>2.88                         | 33<br>33<br>Seizure.<br>Do.<br>Do. |

Referring to Table IV, the preferred grease composition #15 without extreme pressure additives will not pass the Timken test. Greases 16 through 19 show that dibenzyl disulfide or tricresyl phosphate alone are not adequate to meet the test when incorporated in the preferred grease #15. Chassis grease A, a lubricant manufactured by ordinary methods, does not pass the test with

or without additives, as shown by greases 20, 21, 22, and 23. The combination of lead naphthenate, air-blown asphalt and sulfur or lead naphthenate and additive C also failed to carry grease #15 through the Timken test as shown by greases number 25 and 28. Greases 26 and 27, the latter being the preferred formulation since the degree of sulfur activity was optimum, represent a combination which passes the Timken extreme pressure test.

In preparing these extreme pressure greases, the extreme pressure additives may be incorporated into a finished lime-base grease composition in amounts sufficient to attain the desired characteristics or may be incorporated during the steps of preparation. The preferred procedure comprises adding the lead naphthenate and sulfurized terpene after the step of adjusting the free alkalinity, while the grease is at 150-160° F. with continued agitation. After the elapse of about one hour from the time of addition of the wash-oil, the agitation is stopped and the product cut to desired consistency.

Although the invention has been described by disclosure of specific embodiments exemplifying the preferred method of preparation and the preferred compositions, the only limitations to be placed upon the scope of the invention appear in the appended claims.

What is claimed is:

1. A lubricating grease comprising the following ingredients in weight per cent:

|                                                                                               |           |
|-----------------------------------------------------------------------------------------------|-----------|
| C <sub>16</sub> to C <sub>18</sub> animal fatty acids                                         | 8-9       |
| 30 Hydrated lime                                                                              | 1.5-1.7   |
| Caustic soda                                                                                  | 0.01-0.20 |
| Phenol extract from bright stock manufacture,<br>API gravity 8.6° to 15.4°, viscosity at 100° |           |
| F. of 15,000 to 145,000 SUS                                                                   | 60-65     |
| 35 Solvent refined neutral lubricating oil                                                    | 24-30     |
| Water                                                                                         | 0.2-0.35  |

2. A lubricating grease in accordance with claim 1 in which the fatty acid is selected from the group consisting of stearic acid and palmitic acid and mixtures thereof.

3. A lubricating grease comprising the following ingredients in weight per cent:

|                                                                                                                       |       |
|-----------------------------------------------------------------------------------------------------------------------|-------|
| C <sub>16</sub> to C <sub>18</sub> animal fatty acids                                                                 | 8.40  |
| 45 Hydrated lime                                                                                                      | 1.60  |
| Caustic soda                                                                                                          | 0.06  |
| Phenol extract from bright stock manufacture,<br>API gravity about 12.6°, viscosity at 100° F. of<br>about 36.410 SUS | 62.77 |
| 50 Viscosity 200 SUS at 100° F. Mid-Continent sol-<br>vent refined neutral lubricating oil                            | 26.89 |
| Water                                                                                                                 | 0.28  |

4. The method of preparing a lime-base grease comprising heating and agitating about 6,300 parts of phenol extract having an API gravity about 8.6° and a viscosity at 100° F. of about 36,410 SUS obtained from the manufacture of lubricating oil bright stock in a reaction kettle to about 160° to 180° F., said extract containing a predominance of aromatic hydrocarbons, preparing a lime-

60 dominance of aromatic hydrocarbons, preparing a lime-oil slurry of about 500 parts of solvent refined neutral lubricating oil having a viscosity of 200 SUS at 100° F. and about 160 parts of hydrated lime by thorough mixing and dispersion, adding about 28 parts of water containing about 7 parts of sodium hydroxide to the phenol extract, slowly adding about 80 parts of the lime-oil slurry to the phenol extract and sodium hydroxide mixture, heating and agitating the mixture until a maximum temperature of 203° F. is reached, adding about 1,700 parts of said solvent refined neutral lubricating oil and 855 parts of animal fatty acids having 16 to 18 carbon atoms per molecule while maintaining the temperature at 200° to 203° F., adding the remaining portion of lime-oil slurry to the mixture, correcting the free alkalinity to within 0.01 to 0.10 percent.

11

diluting to attain the desired quick-chill penetration, and  
packaging the grease.

**References Cited in the file of this patent****UNITED STATES PATENTS**

1,619,352 McKee ----- Mar. 1, 1927

1,699,961  
2,038,689  
2,058,236  
2,245,772  
5 2,312,725  
2,326,596  
2,398,075

12

Finlay ----- Jan. 22, 1929  
Taylor et al. ----- Apr. 28, 1936  
Kaufman et al. ----- Oct. 20, 1936  
Gothard et al. ----- June 17, 1941  
Morway et al. ----- Mar. 2, 1943  
Zimmer et al. ----- Aug. 10, 1943  
Brunstrum et al. ----- Apr. 9, 1946